# EUROPEAN PATENT SPECIFICATION

(11) **EP 0 248 396 B1**
(45) Date of publication and mention of the grant of the patent: **28.04.1993**
(21) Application number: 87107945.5
(22) Date of filing: 02.06.1987
(51) Int. Cl.: C22B 34/14, C22B 9/16

(54) **Combined electron beam and vacuum arc melting for barrier tube shell material**
Verfahren zum Herstellen von Hüllmaterial durch kombiniertes Umschmelzen mit Elektronenstrahlen und Vakuum-Lichtbogen
Procédé pour la fabrication de matériaux de gainage par une combinaison d'une fusion par un faisceau d'électrons et par arc sous vide

(30) Priority: 05.06.1986 US 871183
(43) Date of publication of application: 09.12.1987
(73) Proprietor: WESTINGHOUSE ELECTRIC CORPORATION, Pittsburgh Pennsylvania 15222 (US)
(72) Inventor: Worcester, Samuel Austin, Ogden, UT 84403 (US); Woods, Charles Robert, Ogden, UT 84403 (US)
(74) Representative: Stratmann, Ernst, Dr.-Ing.

(56) References cited:
- EP-A- 0 146 314
- DE-B- 1 121 281
- FR-A- 1 331 472
- JP-A- 5 667 788
- US-A- 3 091 525
- US-A- 3 219 435
- US-A- 4 108 644
- Winkler et al., VACUUM METALLURGY, 1971, Elsevier, Amsterdam-London-New York; pp. 270, 271, 618, 619, 625, 626#

## Description

This invention relates to the production of purified zirconium.

The conventional process for making zirconium metal utilizes a fluidized bed process in which the ore is subjected to a chlorination step which produces a relatively impure, hafnium-containing zirconium tetrachloride and by-product silicon tetrachloride (which by-product is relatively easily separated). The hafnium and zirconium containing material is then subjected to a number of purifying operations and also a complex hafnium separation operation. These operations result in purified oxides of zirconium and hafnium, which, of course, are maintained separate. The purified oxides are separately chlorinated. Zirconium and hafnium are commonly reduced from the chloride by means of a reducing metal, typically magnesium. At the present time, the commercial processes are batched-type processes. U.S. Patent Specification No. 3,966,460, for example, describes a process of introducing zirconium tetrachloride vapor onto molten magnesium, with the zirconium being reduced and traveling down through the magnesium layer to the bottom of the reactor and forming a metallic sponge. The metallic sponge (containing remaining chloride and some remaining excess reducing metal) is then placed in a distillation vessel for removal of the remaining salt and reducing metal by high temperature vacuum distillation. The sponge material is generally crushed, screened and pressed into electrodes for vacuum arc melting. Particularly, the material is multiple (typical double or triple) vacuum arc melted to provide ingots which are then further fabricated into various shapes. Most of the zirconium currently is used to produce Zircaloy.

Commercial nuclear reactors generally have used Zircaloy tubes as cladding material to contain the uranium dioxide fuel. Generally a Zircaloy ingot is processed into a so-called "trex" and pilgering operations are used to reduce the trex inside diameter and wall thickness to size. Ultra-pure zirconium has been proposed for a liner for the inside surface of Zircaloy tubing which is used as a cladding for nuclear fuel and is described in, for example, U.S. Patent Specification No. 4,372,817 (Armijo et al.). A similar use of moderate purity material is proposed in U.S. Patent Specification No. 4,200,492 (Armijo et al.). The ultra-pure zirconium material described has been purified by iodide cells to produce so called "crystal bar" material. This rather expensive crystal bar processing is performed after reduction and is described, for example, in U.S. Patent Specification No. 4,368,072 (Siddal).

EB (electron beam) melting of materials, including zirconium has been discussed in a number of U.S. patent specifications. EB melting has been used to consolidate crushed particles or chips in so called hearth furnaces and to separate impurities by either overflowing floating inclusions (U.S. Patent Specification No. 4,190,404 (Drs et al.)) or to produce an electrode for arc melting (U.S. Patent Specification No. 4,108,644 (Walberg et al.)). A number of U.S. patent specifications have described the EB melting of powders or granules, often producing an ingot in a chilled mold. These powder melting EB patents include U.S. Patent Specification No. 2,942,098 (Smith); 2,960,331 (Hanks); 2,963,530 (Hanks et al.); 2,997,760 (Hanks et al.); 2,935,395 (Smith); and 4,482,376 (Tarasescu et al.). Electron beam zone refining using multiple passes is described in U.S. Patent Specification No 3,615,345 (King).

EB melting using a consumable feed, "electrode" to produce an ingot collected in a chilled mold has also been discussed in a number of U.S. patent specifications, including U.S. Patent Specifications 3,087,211 (Howe); 3,226,223 (Bussard et al.); 2,880,483 (Hanks et al.); and 4,130,416 (Zaboronok et al.). U.S. Patent Specification No. 3,219,435 (Gruber et al.) shows a commercial type EB furnace utilizing multiple beams. Typically the beams are directed to the surface of the molten pool and are continually swept across the pool surface to avoid overheating of any single portion of the pool surface. U.S. Patent Specification No. 3,091,525 (D'A. Hunt) describes adding a small amount of zirconium, for example, to hafnium, for example and melting in an EB furnace to deoxidize the hafnium. Japanese application 1979-144789 Kawakita, published as patent publication 1981-67788 describes the use of a very small ingot with a high power density and ultra slow melting to produce a deep molten pool to produce a high purity ingot directly usable for lining of Zircaloy tubing for nuclear reactor applications. Such laboratory sized apparatus with its high powered consumption and very low throughput is, of course, not practical for commercial production.

Accordingly, a process for producing zirconium in purified form for use in lining the interior of zirconium alloy fuel element cladding comprises reducing zirconium tetrachloride to produce a sponge of metallic zirconium which is distilled to generally remove residual magnesium and magnesium chloride, and melting the distilled sponge to produce an ingot of non-crystal bar material, by forming said distilled sponge into a consumable electrode by pressing crushed virgin sponge into the form of an electrode and then welding an end fitting to the electrode; melting said consumable electrode in a multiple swept beam electron furnace with a feed rate of from 2,5 cm to 51 cm (1 to 20 inches) per hour to form an intermediate ingot, the intermediate ingot having a diameter of greater than 12,7 cm (5 inches); and vacuum arc melting said intermediate ingot to produce a homogeneous final ingot having 50 - 300 ppm iron, 250 - 450 ppm oxygen and 500 - 1000 ppm of total impurities.

This is a process for making very pure and very homogeneous material for use in the lining of the interior of zirconium alloy fuel element cladding. Generally this process provides material much purer than the so called sponge material and almost as pure as the crystal bar material, at a fraction of the cost of crystal bar material. Generally purified zirconium produced according to the present invention has oxygen in the 250-450 ppm range (and preferably less than about 350) and iron in the 50-300 ppm range. Total impurities are generally in the 500-1000 ppm range (total impurities for these purposes generally comprise the elements listed in the afore-mentioned U.S. Patent Specification No. 4,200,492).

Preferably the energy input via the electron beams is maintained to a moderate level such that the molten pool on the upper portion of the intermediate ingot has a depth of less than about one fourth of the ingot diameter, thus lowering power costs. Preferably an argon sweep is provided in the electron beam furnace during melting. Multiple passes may be made both through the EB furnace and the vacuum arc furnace.

The distilled zirconium sponge is formed into a consumable electrode for use in a production EB furnace. A production furnace is generally shown in the afore-mentioned U.S. Patent Specification No. 3,219,435, but with the multiple beams being constantly swept across the surface of the molten pool (as defined herein, a production EB furnace has an output "intermediate" ingot having a diameter greater than five inches, and generally greater than six inches. Generally, this consumable electrode for EB melting is formed by pressing crushed virgin sponge (not recycle scrap). The compact and an appropriate end fitting are welded to form the consumable electrode.

The consumable EB electrode is melted in a production electron beam furnace with a feed rate of from 2.54 - 50.8 cms per hour (1 to 20 inches per hour). It has been found that small amounts of residual magnesium chloride remain in the electrode and absorb some moisture. Melting at faster than 50.8 cms (20 inches) per hour results in this moisture reacting to oxidized zirconium and thus causing an unacceptably high oxygen level in the product. Conversely too slow a melting rate, while possibly removing some oxygen from the molten pool (as described in the afore-mentioned Japanese patent publication 1981-67788) is uneconomical. It should be noted that significant oxygen removal from the molten pool takes considerable superheating of the molten pool and much slower melting rates and thus this invention provides for no significant oxygen removal from the molten pool. It has also been found that the iron impurity level is generally reduced by about a factor of two, each pass through the EB furnace (that is, when the intermediate ingot formed during the first EB melting pass is used as the consumable electrode for a second EB melting, the iron level is reduced by another factor of approximately 2). It has also been found that the level of other common impurities, for example aluminum and chromium, are also reduced by each pass through the EB furnace. It should also be noted that, as the residual magnesium chloride is generally removed during the first EB melting, there is minimal absorbed moisture on the second pass and thus somewhat faster speeds may be used after the first EB pass.

Generally an argon sweep is provided in the electron beam furnace during melting. It is felt that this helps remove moisture which has been vaporized off the electron from the furnace, minimizing contamination of the output intermediate ingot. Preferably the argon sweep is at a flow of 10,000-1,000,000 liters per second, with the liters measured at a pressure of 1,33·10⁻⁵ Pa (10⁻⁵ Torr) (rather than at standard conditions). The argon sweep can be established, for example, with pumps capable of handling 60,000 liters per second and with a pressure of 1,33·10⁻⁵ Pa (10⁻⁵ Torr) measured with no argon flow, by controlling argon introduction to a rate to raise the pressure to approximately 1,33·10⁻⁴ Pa (10⁻⁴ Torr).

It should be noted that the sponge used to form the consumable electrode is generally virgin material (as opposed to recycled scrap or turnings) and preferably is selected high quality material and generally selected for low oxygen content.

Generally, after EB melting, the material is arc melted (and preferably double arc melted or even triple arc melted) to homogenize the impurity distribution. It has been found that in production EB furnaces, with their relatively shallow molten pool (the molten pool being shallow both in comparison to arc melting, where the molten pool is typically about twice the ingot diameter and in comparison to non-multiple swept beam, laboratory type furnaces where the fixed single beam covers essentially the entire surface of the molten pool and produces molten pools of about one diameter in depth) do not produce a homogeneous product. The zirconium material beneath the molten pool is, of course, solid, and can be slowly withdrawn as material from the electrode drips into the pool, as it is known in the prior art.

Thus, on a production EB furnace, the shallow molten pool results in a non-homogeneous product, and only by following such melting with vacuum arc melting can a homogeneous product be obtained. Conversely, non-swept beam EB furnaces having very high power costs for very low throughput, are impractical for commercial applications. This invention lowers oxygen by removing at least some of the moisture prior to melting while the laboratory type of EB furnace is generally removing oxygen from the molten pool.

## Claims

1. A process for producing zirconium in purified form for use in lining the interior of zirconium alloy fuel element cladding which comprises reducing zirconium tetrachloride to produce a sponge of metallic zirconium which is distilled to generally remove residual magnesium and magnesium chloride, and melting the destilled sponge to produce an ingot of non-crystal bar material,
by
a) forming said distilled sponge into a consumable electrode by pressing crushed virgin sponge into the form of an electrode and then welding an end fitting to the electrode;
b) melting said consumable electrode in a multiple swept beam electron furnace with a feed rate of from 2,54 cm (1 inch) to 50,8 cm (20 inches) per hour to form an intermediate ingot, the intermediate ingot having a diameter of greater than 12,7 cm (5 inches);
c) and vacuum arc melting said intermediate ingot;
thereby to produce a homogeneous final ingot having from 50 to 300 ppm iron, from 250 to 450 ppm oxygen and from 500 to 1000 ppm of total impurities.

2. A process according to claim 1, characterized in that the intermediate ingot has on its upper portion a molten pool of less than one fourth of an ingot diameter in depth.

3. A process according to claim 1 or 2, characterized in that an argon sweep is provided in the electron beam furnace during said melting.

4. A process according to claim 3, characterized in that the argon sweep is at a flow of 10,000-1,000,000 liters per second, measured at a pressure of 1,33·10⁻⁵ Pa (10⁻⁵ Torr),

5. A process according to any of claims 1 to 4, characterized in that multiple passes are made through the electron beam furnace.

6. A process according to nay of claims 1 to 5, characterized in that multiple passes are made through the vacuum arc melting.

## Patentansprüche

1. Ein Verfahren zur Erzeugung von Zirconium in gereinigter Form zur Verwendung in der Auskleidung des Inneren einer Zirconiumlegierungsbrennstoffelementummantelung, die das Reduzieren von Zirconiumtetrachlorid zur Erzeugung eines Schwammes von metallischen Zirconium umfaßt, welches destilliert wird, um allgemein Restmagnesium und Magnesiumchlorid zu entfernen, und Schmelzen des destillierten Schwammes zur Erzeugung eines Barrens aus nicht kristallisiertem Barrenmaterial,
durch
a) Formen des destillierten Schwammes zu einer verbrauchbaren Elektrode durch Pressen von zerdrücktem jungfräulichem Schwamm zu der Form einer Elektrode und dann Schweißen eines Endanschlusses an die Elektrode;
b) Schmelzen der verbrauchbaren Elektrode in einem Vielfachverschwenkungsstrahlelektronenofen mit einer Zufuhrrate von 2,54 cm (1 Zoll) bis 50,8 cm (20 Zoll) pro Stunde, um einen Zwischenbarren zu erzeugen, wobei der Zwischenbarren einen Durchmesser aufweist, der größer ist als 12,7 cm (5 Zoll);
c) und Vakuumlichtbogenschmelzen des Zwischenbarrens; um dadurch einen homogenen endgültigen Barren zu erzeugen, der 50 bis 300 ppm Eisen, 250 bis 450 ppm Sauerstoff und 500 bis 1000 ppm gesamte Unreinheiten besitzt.

2. Ein Verfahren nach Anspruch 1, gekennzeichnet dadurch, daß der Zwischenbarren auf seinem oberen Teil einen geschmolzenen Teich mit einer Tiefe von weniger als einem Viertel des Barrendurchmessers aufweist.

3. Ein Verfahren nach Anspruch 1 oder 2, dadurch gekennzeichnet, daß eine Argonspülung in dem Elektronenstrahlofen während des Schmelzens vorgesehen ist.

4. Ein Verfahren nach Anspruch 3, dadurch gekennzeichnet, daß die Argonspülung eine Strömung von 10.000 bis 1.000.000 Liter pro Sekunde ist, gemessen bei einem Druck von 1,33 X 10⁻⁵ Pa (10⁻⁵ Torr).

5. Ein Verfahren nach einem der Ansprüche 1 bis 4, dadurch gekennzeichnet, daß Vielfachdurchläufe durch den Elektronenstrahlofen gemacht werden.

6. Ein Verfahren nach einem der Ansprüche 1 bis 5, dadurch gekennzeichnet, daß Vielfachdurchläufe durch den Vakuumlichtbogenofen gemacht werden.

## Revendications

1. Procédé pour produire sous une forme purifiée du zirconium destiné au garnissage de l'intérieur de gaines en alliage de zirconium pour éléments combustibles, comprenant la réduction de tétrachlorure de zirconium pour produire une éponge de zirconium métallique qui est distillée pour éliminer globalement le magnésium et le chlorure de magnésium résiduels, et la fusion de la éponge distillée pour produire un lingot de matière amorphe en barre,
par
a) la réalisation d'une électrode consommable à partir de ladite éponge distillée en comprimant de l'éponge vierge broyée pour lui donner la forme d'une électrode, puis le soudage d'un embout à une extrémité de l'électrode;
b) la fusion de ladite électrode consommable dans un four à balayage multiple par faisceau d'électrons, avec une Vitesse d'avance comprise entre 2,54 cm (1 pouce) et 50,8 cm (20 pouces) par heure pour former un lingot intermédiaire, le lingot intermédiaire ayant un diamètre supérieur à 12,7 cm (5 pouces);
c) et le soudage à l'arc sous vide dudit lingot intermédiaire;
pour produire de ce fait un lingot final homogène contenant entre 50 et 300 ppm de fer, entre 250 et 450 ppm d'oxygène et entre 500 et 1 000 ppm d'impuretés totales.

2. Procédé selon la revendication 1, caractérisé en ce que le lingot intermédiaire a, sur sa partie supérieure, une masse fondue d'une profondeur inférieure à un quart de diamètre de lingot.

3. Procédé selon la revendication 1 ou 2, caractérisé en ce qu'un balayage à l'argon est réalisé pendant ladite fusion dans le four à faisceau d'électrons.

4. Procédé selon la revendication 3, caractérisé en ce que le balayage à l'argon s'effectue sous un flux de 10 000 à 1 000 000 litres/seconde, mesuré à une pression de 1,33·10⁻⁵ Pa (10⁻⁵ torr).

5. Procédé selon l'une quelconque des revendications 1 à 4, caractérisé en ce que plusieurs passes sont effectuées dans le four à faisceau d'électrons.

6. Procédé selon l'une quelconque des revendications 1 à 5, caractérisé en ce que plusieurs passes sont effectuées dans le four de fusion à arc sous vide.
